# EUROPEAN PATENT SPECIFICATION

(11) **EP 2 625 252 B1**
(45) Date of publication and mention of the grant of the patent: **16.09.2015**
(21) Application number: 11797048.3
(22) Date of filing: 03.10.2011
(51) Int. Cl.: C10L 1/02, C10L 10/00

(54) **USE OF RAPE METHYL ESTER AS PRECIPITATION-INHIBITING FUEL ADDITIVES**
VERWENDUNG VON RAPSÖLMETHYLESTERN ALS KRAFTSTOFFADDITIF ZUR VERHINDERUNG VON NIEDERSCHLAGEN
UTILISATION D'ESTER METHYLIQUE DE COLZA POUR CARBURANTS AFIN D'INHIBITER DES PRECIPITATIONS

(30) Priority: 06.10.2010 SE 1051044
(43) Date of publication of application: 14.08.2013
(73) Proprietor: Scania CV AB, 151 87 Södertälje (SE)
(72) Inventor: HÖGGREN, Lena, S-647 35 Mariefred (SE)
(74) Representative: Scania CV AB
(86) International application number: PCT/SE2011/051174
(87) International publication number: WO 2012/047157

(56) References cited:
- EP-A1- 2 233 552
- DATABASE WPI Week 200711 Thomson Scientific, London, GB; AN 2007-102882 XP002667450, & CN 1 793 292 A (SHI S) 28 June 2006 (2006-06-28)
- MAKAREVICIENE: "Investigation of the characteristics of Multicomponent Biodiesel Fuel (D_FAME-E) for Practical Use in Lithuania", ENERGY FUELS, vol. 24, 30 December 2009 (2009-12-30), pages 1365-1373, XP002667451,

## Description

This invention relates to use of a composition containing rape methyl ester (RME) as a precipitation-inhibiting fuel additive in cases where precipitation occurs in the fuel system of ethanol-powered engines and arises from motor oils.

### Background to the invention

Many motor vehicles are now run on ethanol-based fuels. Certain vehicles, e.g. buses, have engines which work according to the diesel principle and use ethanol as fuel.

One of known problems with the fuel system of such ethanol buses/ethanol engines is rapid formation of a sticky precipitate which then obstructs the fuel filter and causes blockages in the fuel return line etc. This sticky precipitate is formed as a result of motor oil additives, inter alia PIBSI (polyisobutylene succinimide), precipitating in the ethanol system. This component is used as a dispersant in motor oil with the object of keeping particles of soot or metals floating in solution.

There is currently no substitute for PIBSI, so the formation of said sticky precipitate still occurs when motor oil and alcohols come into mutual contact.

A known practice from WO 2007053787 (Lubrizol) and WO 2008082916 (Lubrizol) is to add to a fuel, which may be ethanol, a friction modifier which contains a substance chosen from among an alkoxylated fatty amine, a fatty acid or derivatives thereof, and mixtures thereof for use in various types of fuels, including ethanol. The desired effect is that the additives result in less friction in the engine, but also that the cleaning effect and proper functioning at low temperatures are mentioned.

Prior art does however not deal with the problem of the formation of sticky precipitates pertaining to such fuel and consequently does not propose any additives specifically intended to solve the problem.

### Summary of the invention

The present invention aims at eliminating or in any case reducing the presence of sticky precipitates in the fuel system of engines run on ethanol-based fuels.

This object is achieved by usingrape methyl ester (RME), as a fuel additive to prevent formation of sticky precipitates in an engine which is run on an ethanol-based fuel and which has a motor oil additive in the form of a dispersant. This additive to the alcohol fuel serves as a means of dissolving or preventing sticky precipitates and may thereby reduce them.

The addition of RME is therefore not to serve as a friction modifier as in prior art.

The disadvantage of RME is its poor solubility at low temperatures. It has now surprisingly been found that an emulsifier (Ethomeen O/ 12™; AKZO NOBEL) which is an amine and already normally present in ethanol fuels, causes RME to precipitate less readily at low temperatures.

In an embodiment, the additive is used in combination with an amine, preferably bis-(2-hydroxyethyl)-oleyl amine.

Combining these components in amounts corresponding to 1 wt% RME (rape methyl ester) and 1 wt% Ethomeen O / 12 ™, in cases where they are present in the ethanol fuel, results in an optimum combination. With this mixture, RME does not precipitate at low temperatures such as down to -28°C (RME has a cloud point of -10 °C to -14 °C).

Fatty acid alkyl ester contents in the fuel may range between 1 wt% and 3 wt%, with a preferred content of 1 wt%, based on the total weight of the composition.

The invention thus minimises precipitation of oil additives in the fuel system of an ethanol engine which works according to the diesel principle.

A further advantage of the invention is that it works even in cold climates.

Another aspect of the disclosure proposes a fuel containing 91.2 - 98.5% ethanol, 0.5 - 1.1 % bis-(2-hydroxyethyl)-oleyl amine and 1 - 2 % RME and possibly other additives up to 100%.

A further aspect of the invention relates to a fuel additive composition comprising a mixture of RME and bis-(2-hydroxyethyl)-oleyl amine in a weight ratio of 3:1 to 1:1.

### Detailed description

The invention relates to use of a fatty acid methyl and fatty acid ethyl esterrape methyl ester (RME) as additive to ethanol fuels for engines which work according to the diesel principle. This additive reduces the formation of sticky precipitates in the engine's fuel system.

For certain vehicles the fuel needs at present to contain at least 91.2 wt% ethanol, but the invention is also applicable to other ethanol contents, down to 90 wt% but even down to 85 wt%.

The fuel injectors in an ethanol engine comprise a number of movable parts which need lubrication. Such lubrication is provided via ducts which are situated within the material of the injectors and which lead to the lubrication points, e.g. the piston which feeds fuel to the engine and moves to and fro in a bore. Small amounts of lubricant unavoidably pass through seals and penetrations in the movable parts. Hence additives such as PIBSI (polyisobutylene succinimide) may also enter the fuel system, in which they form sticky precipitates and may cause stoppages.

The inventors have surprisingly now discovered that a known fuel additive in the form of RME causes said sticky precipitates to dissolve or quite simply be prevented from forming.

Without wishing to tie themselves to any theory, the inventors consider it likely that PIBSI (polyisobutylene succinimide) is quite simply dissolved and kept in solution in the fuel as a result of the additive according to the invention.

The additive takes the form of RME (rape methyl ester) which is a form of FAME (fatty acid methyl ester). Rape oil is made by pressing rapeseed and is a mixture of various different fatty acids. 100 grams of rape oil contains 6 g of saturated fatty acids, 62 g of monounsaturated fatty acids, 31 g of polyunsaturated fatty acids and 1 g of other fats. RME is made by esterification of rape oil with methanol and potassium hydroxide.

In a preferred embodiment, the ester is used together with an amine, preferably bis-(2-hydroxyethyl)-oleyl amine, which prevents the ester from precipitating at low temperatures.

The invention may be implemented in various ways.

In a first aspect, the ester is used alone as an additive which is provided separately and is put into a vehicle's fuel tank after it has been replenished with ethanol fuel. In this case the fuel must therefore already contain amine to ensure that low temperature operation is possible. It is here also conceivable that the fuel supplier might add RME from the outset before the fuel reaches the customer.

Ethanol fuels today often already contain said amine, with the result that adding a correct amount of esters would suffice to achieve the desired effect according to the invention.

Alternatively, in a second aspect of the invention, it is possible to propose a composition comprising two components, viz. an ester and an amine in suitable proportions.

A further aspect of the dislosure proposes a fuel which already contains not only ethanol but also a specific amount of ester and a specific amount of amine.

The table below summarises a number of experiments with different contents of the various components in an ethanol fuel, showing the compositions with which the additive does not precipitate.

These experiments use rape methyl ester (RME) as precipitation-inhibiting additive and an ethanol fuel (ED 95) with an amine in the form of Ethomeen 0 / 12™ (commercially available from Akzo Nobel) with the commercial name bis-(2-hydroxyethyl)-oleyl amine.

**Table 1**

| Ethomeen 0/12 content | RME wt% | Temperature | Precipitation |
|---|---|---|---|
| 1 wt% | 5 wt% | - 28 °C | Yes |
| 1 wt% | 3 wt% | - 28 °C | No |
| 1 wt% | 2 wt% | - 28 °C | No |
| 1 wt% | 1 wt% | - 28 °C | No |

Table 1 shows that high ester contents do not work, but that precipitation does not occur with 1 wt% amine (Ethomeen 0/ 12) and 1 - 2 wt-% RME in ED 95 at -28°C.

**Table 2**

| Ethomeen 0/12 content | RME wt% | Temperature | Precipitation |
|---|---|---|---|
| 0 wt% | 1 wt% | - 28 °C | Obscure |
| 0 wt% | 2 wt% | - 28 °C | Obscure |
| 0 wt% | 3 wt% | - 28 °C | Yes |

Table 2 shows that with no Ethomeen 0/12 in the fuel, RME precipitates in cold conditions.

**Table 3**

| Ethomeen 0/12 content | RME wt% | Temperature | Precipitation |
|---|---|---|---|
| 0.25 wt% | 1 wt% | - 28 °C | Obscure |
| 0.50 wt% | 1 wt% | - 28 °C | Yes |

Table 3 shows a lower limit for Ethomeen 0/12 content in that more than 0.50 wt% Ethomeen in the fuel is required for RME not to precipitate in cold conditions.

To sum up, it may be stated that in combination with 1 wt% Ethomeen 0/ 12 it is therefore possible to use RME contents of between 1 and 3 wt% in ED 95 without precipitation occurring in cold conditions.

The invention is illustrated by the following examples.

ED 95 is an ethanol fuel which contains at least 91.2 wt% ethanol, about 5.0 wt% of ignition improver and further components up to 100%.

### EXAMPLE 1 (not according to the invention)

The fuel injectors (Scania Duel Rail) for an ethanol engine (Scania DC9 E02) which works according to the diesel principle are supplied with ED 95 fuel of standard type. It is found that the nozzle needle runs sluggishly in its bore because the needle becomes sticky. The deposit forms and builds up over time.

### EXAMPLE 2

The same engine as in example 1 is supplied with ED 95 fuel of standard type but with an additive according to the invention. The nozzle needle is found to run easily in its bore because the needle does not become sticky.

## Claims

1. Use of rape methyl ester (RME) to prevent formation of sticky precipitates in an engine, which is run on an ethanol-based fuel and has a motor oil additive in the form of a dispersant where the engine works according to the diesel principle, and that the rape methyl ester is a fuel additive used to prevent formation of sticky precipitates, and where, in case the engine is to be used in temperature conditions in which the RME precipitates, the rape methyl ester is used in combination with an amine.

2. Use according to claim 1, in combination with an amine.

3. Use according to claim 1 or 2, in which the amine is bis-(2-hydroxyethyl)-oleyl amine.

4. A fuel additive composition containing rape methyl ester (RME) and bis-(2- hydroxyethyl)-oleyl amine in a weight ratio of 3: 1 to 1: 1.

## Patentansprüche

1. Verwendung eines Rapsmethylesters (RME) zum Verhindern einer Bildung von klebrigen Ausscheidungsprodukten in einem Motor, der mit einem ethanolbasierten Kraftstoff betrieben wird und einen Motorölzusatz in Form eines Dispersionsmittels aufweist, wobei der Motor nach dem Diesel-Prinzip funktioniert, wobei der Rapsmethylester ein Brennstoffadditiv zum Verhindern der Bildung von klebrigen Ausscheidungsprodukten ist, und wobei, falls der Motor dazu vorgesehen ist, unter Temperaturbedingungen genutzt zu werden, unter denen der RME kondensiert, der Rapsmethylester in Verbindung mit einem Amin verwendet wird.

2. Verwendung nach Anspruch 1, in Verbindung mit einem Amin.

3. Verwendung nach Anspruch 1 oder 2, bei der das Amin ein Bis-(2-Hydroxyethyl)-oleylamin ist.

4. Eine Brennstoffadditivzusammensetzung, die einen Rapsmethylester (RME) und ein Bis-(2-Hydroxyethyl)-oleylamin mit einem Gewichtsverhältnis von 3:1 bis 1:1 umfasst.

## Revendications

1. Utilisation d'ester méthylique de colza (EMC) pour prévenir la formation de précipités collants dans un moteur qui fonctionne au carburant à base d'éthanol et a un additif d'huile moteur sous forme de dispersant, où le moteur fonctionne selon le principe du diesel, et l'ester méthylique de colza est un additif de carburant utilisé pour prévenir la formation de précipités collants, et où, dans le cas où le moteur doit être utilisé dans des conditions de température dans lesquelles l'EMC précipite, l'ester méthylique de colza est utilisé en combinaison avec une amine.

2. Utilisation selon la revendication 1, en combinaison avec une amine.

3. Utilisation selon la revendication 1 ou 2, où l'amine est la bis-(2-hydroxyétlryl)oléylamine.

4. Composition d'additif de carburant contenant de l'ester méthylique de colza (EMC) et de la bis-(2-hydroxyéthyl)oléylamine dans un rapport pondéral de 3:1 à 1:1.
